

## UNITED STATES PATENT OFFICE

CAMILLE DREYFUS, OF NEW YORK, N. Y.

## PRODUCT FROM ORGANIC DERIVATIVES OF CELLULOSE

No Drawing.

Application filed November 4, 1926. Serial No. 146,287.

This invention relates to a new and improved fabric or textile material with moire effects which are permanent in nature.

It is well known that moire effects on silks, 5 linens etc., are obtainable by subjecting ribbed fabrics to heat and pressure under certain conditions. Moire effects on plain or satin weave fabrics have also been obtained by subjecting such fabrics to the action of 10 engraved rollers under heat and pressure.

The moire effects obtained by the above processes on such materials, however, have the drawback that they are not permanent. On continued wear or upon washing, laundering 15 etc., the moire effect gradually lessens and finally disappears completely. The applicant has now discovered that permanent effects are obtained when certain materials are treated by known processes. He has found 20 that if fabrics or textile materials made wholly or largely from organic derivatives of cellulose are subjected to any of the known processes for obtaining moire effects, beautiful and permanent effects can be obtained on 25 these fabrics. Fabrics made from cellulose acetate, cellulose propionate, or ethyl cellulose etc., give excellent results.

Moire Française and moire Renaissance are obtainable on cellulose acetate fabrics, 30 the markings being very pronounced and beautiful. Fine moire effects were also obtained on such fabrics by embossing appropriate designs thereon under heat and pressure by means of engraved rollers. Fabrics 35 marked by either of the above methods were washed, laundered, etc., with no visible effect on the moire, differing very strikingly from silk or other fabrics in this respect. This is true in spite of the fact that such fabrics need 40 not be subjected to as high a heat when imparting the moire effects thereto as is necessary to impart moire effects to silk or similar fabrics. Very pleasing results are obtained by producing moire effects on ribbed 45 fabrics containing the organic derivatives of cellulose such as cellulose acetate.

Excellent results have been obtained with cellulose acetate fabrics but the invention is not to be considered as limited to such fabrics. 50 It includes within its scope any fabrics made

wholly or partially from organic derivatives of cellulose having permanent moire effects and the invention is to be construed as limited only by the scope of the appended claims.

Having described my invention, what I 55 claim and desire to secure by Letters Patent is:

1. A textile material comprising individual filaments of organic derivatives of cellulose, at least some of which filaments are permanently deformed and present a moire design 60 which is permanent.

2. A textile material comprising individual filaments of organic esters of cellulose, at least some of which filaments are permanently deformed and present a moire design 65 which is permanent.

3. A textile material comprising individual filaments of cellulose acetate, at least some of which filaments are permanently deformed 70 and present a moire design which is permanent.

4. A fabric comprising individual filaments of organic derivatives of cellulose, at least some of which filaments are permanently deformed and present a moire design which is permanent. 75

5. A ribbed fabric comprising individual filaments of organic derivatives of cellulose, at least some of which filaments are permanently deformed and present a moire design 80 which is permanent.

6. A ribbed fabric comprising individual filaments of organic esters of cellulose, at least some of which filaments are permanently deformed 85 and present a moire design which is permanent.

7. A ribbed fabric comprising individual filaments of cellulose acetate, at least some of which filaments are permanently deformed 90 and present a moire design which is permanent.

In testimony whereof, he has hereunto subscribed his name.

CAMILLE DREYFUS. 95